

# UNITED STATES PATENT OFFICE.

FIN SPARRE, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## ALUMINUM-GLAZED BLACK POWDER.

1,116,944.

Specification of Letters Patent. Patented Nov. 10, 1914.

No Drawing.

Application filed September 20, 1913. Serial No. 790,846.

To all whom it may concern:

Be it known that I, FIN SPARRE, of Wilmington, in the county of New Castle, and in the State of Delaware, have invented a 5 certain new and useful Improvement in Aluminum-Glazed Black Powder, and do hereby declare that the following is a full, clear, and exact description thereof.

My invention relates to an improvement 10 in black gunpowder but has special reference to the coating of granulated black gunpowder, such, for example, as that used in blasting operations.

My invention relates especially, however, 15 to providing a coating for such powder.

Hitherto gunpowder for blasting purposes or for firearms has been manufactured with a coating of graphite, the same having been applied as the last step in the manufacture thereof. Such coating of graphite has 20 been called glazing, inasmuch as its presence provides the powder with a smoother surface and renders the surface thereof glossy.

Textbooks, referring to glazing by the application of a coating of graphite, state that such coating reduces the hygroscopicity of the powder and that it causes the powder to run more easily in the loading machines and 25 that it also assists in obtaining uniform ballistic results in firearms. It has been demonstrated, however, that the use of a coating of graphite renders the powder less hygroscopic to only a negligible degree and, 30 furthermore, that the ease of running in the loading machines and bore holes is not entirely dependent upon the application of a coating of graphite but that this result may also be obtained to an extent sufficient 35 for most purposes by a rubbing of the grains or by tumbling the same in a barrel. It has also been demonstrated that the use of a coating of graphite decreases the strength of the powder.

The object of my invention is to overcome 40 previous disadvantages and in general my invention comprises the production of a coating upon black gunpowder by the use of a pulverized metallic substance containing aluminum. This has the advantage of 45 providing a coating which seems an active constituent of the explosive inasmuch as the aluminum in itself is a desirable component of explosives. It is particularly advanta- 50 geous in aiding quick ignition which is ap-

parent from the fact that the coating material is a good conductor of heat and from the fact that aluminum is a component frequently used in producing explosives. Graphite, on the other hand is a non-active 60 substance as it burns with considerable difficulty compared with the other ingredients present in such powder and as it consequently lowers the rate of ignition. As I have previously pointed out, aluminum has 65 been previously used as an ingredient of explosives. But my invention is directed not to the use of aluminum as a general ingredient of powder of the kind referred to. This will be evident from the small percentage which I ordinarily use in producing 70 black powder in accordance with my invention. Ordinarily the percentage of aluminum which I use is less than 0.5% and the percentage as a rule would be less than 75 0.2%, in view of the fact that only a portion of the pulverized aluminum added to the powder would adhere to the powder.

My invention is directed particularly to the elimination of the objectionable coating 80 agent which has been previously used, graphite, and to providing a coating which does not retard ignition but which in fact hastens the speed of ignition. The coating which I use is more advantageous than 85 graphite for the further reason that it may be applied in a fraction of the time required for the application of graphite, and inasmuch as a smaller quantity of my coating may be used than in the case of graphite. 90

While my invention is capable of being carried out in many different ways, for the purposes of illustration I shall set forth an example of the way in which it may be accomplished. For example, I may use as a 95 coating pulverized aluminum. The aluminum may be applied to the powder in exactly the same manner as graphite is now applied. That is to say, the powder as it comes from the mill may be dried in any 100 suitable manner and the dust separated therefrom. Thereupon the grain may be placed in a barrel revolving at a suitable speed and a small amount of aluminum added to the charge. For example, 2 pounds 105 of aluminum may be added to 1,000 pounds of powder, although a smaller or larger quantity of aluminum may be used according to the degree to which it is desired to change the character of the powder. The 110

charge in the barrel is then revolved for a suitable time as, for example, from fifteen to thirty minutes. I have in some instances, however, been able to apply the aluminum in a shorter time, as for example, ten minutes, but it is conceivable that with different methods the time might be longer even than thirty minutes. During the coating process the materials may or may not be heated as 10 found desirable, as for example according to the humidity of the atmosphere. It may also be found desirable to run the grain directly from the mill into a revolving barrel for a period of time as, for example, a few 15 hours, during which time the powder may if desired be heated, either by warm air being blown into it or by the friction generated by the movement of the powder in the barrel. Thereupon, after the powder has 20 become smooth and has been dried in the barrel, and preferably after the dust has been separated therefrom, the aluminum may be added and applied as indicated above. 25 While I have described my invention above in detail I wish it to be understood

that many changes may be made therein without departing from the spirit of my invention.

I claim:—

1. The process which comprises applying to granulated uncoated black powder a coating of a metallic substance containing aluminum. 30
2. The process which comprises applying to granulated uncoated black powder a coating of aluminum. 35
3. An explosive comprising granulated black powder having a coating of a metallic substance containing aluminum located contiguous to the bodies of black powder in the grains. 40
4. An explosive comprising granulated black powder having a coating of aluminum located contiguous to the bodies of black powder in the grains. 45

In testimony that I claim the foregoing I have hereunto set my hand.

FIN SPARRE

Witnesses:

HAMILTON BRADSHAW,  
JAMES H. LEACH.